

Patented July 2, 1929.

1,719,649

## UNITED STATES PATENT OFFICE.

GEORGE D. CHAMBERLAIN, OF ASHLAND, KENTUCKY, ASSIGNOR TO R. T. VANDERBILT COMPANY, INCORPORATED, OF NEW YORK, N. Y., A CORPORATION OF NEW YORK.

## PICKLING AND CLEANING OF METAL.

No Drawing.

Application filed January 11, 1927. Serial No. 160,525.

This invention relates to the pickling and cleaning of metals, and particularly to the pickling of iron or steel, to remove scale therefrom, although the invention is of more 5 or less general application to the cleaning or pickling of metals such as iron or steel for the removal of oxides or scale therefrom.

The pickling or cleaning of iron or steel is commonly effected by means of acid pickling or cleaning baths which dissolve the scale or oxide from the metal. The pickling baths commonly employed are acid baths which often attack the metal as well as the scale. This action on the metal is undesirable 10 and objectionable, involving not only excessive consumption of acids, but also corrosion or dissolving of metal and tending to give a rough or pitted surface.

The present invention provides an improved bath for pickling or cleaning metals and also an improved process of pickling or cleaning the metal in which the acid pickling bath has incorporated therein a small amount 20 of a condensation product of an organic amine with an aldehyde.

I have found that the addition of a small amount of a suitable condensation product of an aldehyde with an amine prevents or retards or inhibits the attack of the acid 30 pickling bath on the metal without interfering with the removal of scale or oxide by the acid bath and leaves the surface of the cleaned metal in better condition.

The agents which are added to the cleaning or pickling bath, according to the present invention, include various condensation products of amines with aldehydes. Among 35 these may be mentioned condensation products of various aldehydes, such as aldol, acetaldehyde, butyraldehyde, heptaldehyde, furfural, benzaldehyde, etc. with amines. Certain condensation products of aldol with amines are particularly advantageous, such 40 as the condensation product of aldol with alpha-naphthylamine and with certain guanidines such as diphenylguanidine and certain other di-substituted guanidines. Condensation products of guanidines with other aldehydes can also be used, as well as condensation 45 products of other amines with aldehydes. For example, the condensation products of anilin with acetaldehyde, including the condensates produced both in presence and in absence of acid, can be used, or the product 50 formed by the further action of formalde-

hyde on the condensate of acetaldehyde with anilin, among other condensation products may be mentioned the condensation product of heptaldehyde with anilin, of formaldehyde with anilin or with o-toluidine, or furfural with diethyl-amine or with diphenylguanidine, etc.

The acid pickling baths with which the agents mentioned are used may be acid baths such as are commonly employed for pickling 60 or cleaning iron and steel, containing for example, about 10% of sulfuric acid. Such baths are gradually impoverished by the action of the acid in removing the scale or 65 rust and their content of ferrous sulfate increases until the bath becomes too weak or 70 too concentrated in ferrous sulfate for further use. Instead of using sulfuric acid baths, other acid baths can be used, including acid sulfate baths.

The amount of the condensation product added to the bath for carrying out the pickling or cleaning operation can be varied. In general, only a small amount of the condensation product is required, for example, a 75 small fraction of one per cent. In the case of the condensation product of aldol and alpha-naphthylamine, for example, about two pounds of the condensation product can be employed for each ton of 80 60 degree acid used in the pickling bath. A similar or somewhat increased amount of the condensation product of aldol with diphenylguanidine can be similarly used. The condensation product 85 employed should be one which is stable and does not decompose to any objectionable extent in the acid bath.

The carrying out of the pickling or cleaning operation may be the same as in ordinary practice. For example, the pickling can be 90 carried out continuously by passing the material to be pickled, such as wire or sheets, through a number of baths in a regulated manner; or by immersing the article to be 95 pickled in the pickling bath for a suitable period of time. The temperature of the bath can be varied, ordinarily being around 150 to 180° F. The pickling bath may be replenished by the addition of further amounts of acid until the iron sulfate reaches too great 100 a concentration.

The addition of the condensation product to the bath prevents or retards or inhibits the action of the acid bath on the metal without interfering with the removal of scale or 110

oxide. The formation of hydrogen by the action of the acid bath on the metal is also reduced and the evolution of acid mist or fumes also greatly reduced. There is also a saving in the acid as well as a protection of the metal. The reduced amount of action of the acid on the metal and the reduction in amount of hydrogen produced correspondingly reduces the amount of hydrogen absorbed by the metal.

The employment of the condensation product in the pickling or cleaning operation, according to the present invention, involves but small additional expense and results in advantages in operation, economy of acid, protection of the metal from attack, etc., which materially improve the pickling and cleaning operation.

I claim:

20 1. The method of cleaning or pickling metals which comprises subjecting the same to a non-oxidizing mineral acid pickling or cleaning bath and inhibiting the chemical action of the acid on the metal without interfering with the removal of scale or oxide, and thereby reducing the formation of hydrogen and the production of acid fumes and effecting an economy in the acid consumed, by incorporating in the acid bath a small amount of a condensation product of an aldehyde with an amine.

25 2. The method of cleaning or pickling metals which comprises subjecting the same to a non-oxidizing mineral acid pickling or cleaning bath and inhibiting the chemical action of the acid on the metal without interfering with the removal of scale or oxide, and thereby reducing the formation of hydrogen and the production of acid fumes and effecting an economy in the acid consumed, by incorporating in the acid bath a small amount of a condensation product of aldol with an amine.

30 3. The method of cleaning or pickling metals which comprises subjecting the same to a non-oxidizing mineral acid pickling or cleaning bath and inhibiting the chemical action of the acid on the metal without interfering with the removal of scale or oxide, and thereby reducing the formation of hydrogen and the production of acid fumes and effecting an economy in the acid consumed, by incorporating in the acid bath a small amount of a condensation product of aldol with alpha-naphthylamine.

35 4. The method of pickling or cleaning iron or steel which comprises subjecting the same to an acid pickling bath containing sulfuric acid and inhibiting the chemical action of the acid on the metal without interfering with the removal of scale or oxide, and thereby

reducing the formation of hydrogen and the production of acid fumes and effecting an economy in the acid consumed, by incorporating in the acid bath a small fraction of one percent of a condensation product of an aldehyde with an amine. 65

5. The method of pickling or cleaning iron or steel which comprises subjecting the same to an acid pickling bath containing sulfuric acid and inhibiting the chemical action of the acid on the metal without interfering with the removal of scale or oxide, and thereby reducing the formation of hydrogen and the production of acid fumes and effecting an economy in the acid consumed, by incorporating in the acid bath a small fraction of one percent of a condensation product of aldol with an amine. 70

6. The method of pickling or cleaning iron or steel which comprises subjecting the same to an acid pickling bath containing sulfuric acid and inhibiting the chemical action of the acid on the metal without interfering with the removal of scale or oxide, and thereby reducing the formation of hydrogen and the production of acid fumes and effecting an economy in the acid consumed, by incorporating in the acid bath a small fraction of one percent of a condensation product of aldol with alpha-naphthylamine. 80

7. A non-oxidizing mineral acid bath for pickling or cleaning metals which contains a small amount of a condensation product of an aldehyde with an amine.

8. A non-oxidizing mineral acid bath for pickling or cleaning metals which contains a fraction of one percent of the condensation product of aldol with an amine. 95

9. A bath for cleaning or pickling metals which contains sulfuric acid and a small amount of a condensation product of an aldehyde with an amine. 100

10. A bath for cleaning or pickling iron or steel which contains sulfuric acid and a fraction of one percent of a condensation product of aldol with alphanaphthylamine. 105

11. A bath for cleaning or pickling metals which contains sulfuric acid and a condensation product of aldol with alphanaphthylamine. 110

12. A non-oxidizing mineral acid bath for pickling or cleaning metals which contains a condensation product of aldol with an amine.

13. A non-oxidizing mineral acid bath for pickling or cleaning metals which contains a condensation product of aldol with alphanaphthylamine. 115

In testimony whereof I affix my signature.

GEORGE D. CHAMBERLAIN.